

# UNITED STATES PATENT OFFICE.

FRANKLIN R. CARPENTER, OF DENVER, COLORADO, ASSIGNOR OF ONE-HALF TO JOSEPH H. BERRY, OF DETROIT, MICHIGAN.

## PROCESS OF RECOVERING PRECIOUS METALS FROM MATTES CONTAINING THEM.

SPECIFICATION forming part of Letters Patent No. 718,089, dated January 18, 1903.

Application filed September 13, 1902. Serial No. 123,324. (No specimen.)

*To all whom it may concern:*

Be it known that I, FRANKLIN R. CARPENTER, a citizen of the United States, residing at Denver, in the county of Arapahoe and State of Colorado, have invented certain new and useful Improvements in Processes of Recovering Precious Metals from Mattes Containing Them, of which the following is a specification.

10 My invention relates to a process of recovering precious metals from mattes containing them, and especially from mattes produced by smelting dry ores.

15 The treatment of mattes containing precious metals with baths of molten lead is for the purpose of dissolving and concentrating the precious metals in the lead and is well known; but certain difficulties have been found to exist in practicing the process.

20 It has been found in practice that when matte is brought in contact with a molten-lead bath certain reactions take place between the lead and some of the metallic sulfids contained in the matte, resulting in a reduction 25 of the sulfid of the metal or metals and the formation of lead sulfid. The presence of the lead sulfid thus produced in the molten-lead bath prevents its absorbing silver to a variable degree, depending on the quantity of sulfid 30 present, thereby preventing efficient concentration and, what is more serious, a loss of silver in the matte. Moreover, lead sulfid is freely soluble in matte and when formed as above described tends to combine with and 35 be carried away with the discharged matte, thereby causing a loss of lead. Moreover, it has been found that when the bath of metallic lead is contaminated with lead sulfid it absorbs copper from the matte, which makes the 40 subsequent treatment of the lead bullion more difficult. Attempts have been made to overcome these difficulties, as by attempting to reduce the lead sulfid contained in the bath of metallic lead; but this is not found to be efficient. It obviously will not prevent the carrying off of lead by the matte, nor will it more 45 than partially remove the other difficulties.

It is the object of my invention to produce a process by which the precious metals may 50 be effectively recovered from matte contain-

ing them by means of a bath of metallic lead without substantial loss; and to this end my invention consists in causing the matte to be intimately mixed with metallic iron while it is being subjected to the bath of molten lead. 55

In practicing my invention it will generally be found convenient and preferable to form the mixture of metallic iron and matte by dissolving the former in the latter while in a molten condition. The addition may consist 60 of wrought or cast iron or steel scrap, which it has been found will readily dissolve in the molten matte, and the presence or absence of iron sulfid (an ordinary constituent of matte) in no way affects this operation. The quantity of metal to be added may be readily determined by experiment, especially when operating on mattes of substantially constant composition; but the quantity to be used will vary according to the composition of the 70 matte. The quantity of iron to be used may also be determined with safety as that theoretically sufficient to effect the reduction of the metallic sulfids contained in the matte which are capable of being reduced by metallic iron at the temperature to be employed. The solution of the iron in the matte may be effected in any suitable or desired place. For instance, the iron may be dissolved in the molten matte in the forehearth of a cupola 80 or other furnace in which the matte may have been produced or in any furnace in which the matte may have been melted or in a ladle or other vessel used for conveying the molten matte to the lead-bath. It will be found that 85 the iron dissolved in the matte does not segregate on cooling. The matte containing metallic iron is then subjected to the action of a bath of metallic lead in any suitable or desired way, and after the usual treatment there- 90 with it will be found to be completely freed from the precious metals which have become dissolved in the molten lead and no appreciable quantity of lead has been absorbed by the matte. 95

From the preceding description the advantages of my process will be apparent. Instead of attempting to reduce the lead sulfid already formed in the lead-bath I cause the iron to be present at the point where the lead 100

sulfid would otherwise form, and iron sulfid having a higher heat of formation than lead sulfid the latter cannot form in the presence of metallic iron. It will therefore be seen 5 that the objections to the process which have been heretofore pointed out are all obviated.

While I have described the mixture of matte and metallic iron as formed by dissolving scrap in molten matte, I do not desire to limit 10 myself thereto, since the iron may be added in a molten condition, or if the matte contains iron sulfid in sufficient quantities the mixture might be formed by reducing the iron sulfid either before or during the time 15 it is subjected to the lead-bath. If the matte does not contain sufficient iron sulfid, soluble and reducible compounds of iron may be added instead of metallic iron and the mixture treated in the same way as mattes containing iron sulfid.

The reduction of an iron compound contained in the matte is not specifically claimed herein, as the same forms the subject of a

separate application, Serial No. 28,343, filed August 28, 1900.

What I claim herein, and desire to secure by Letters Patent, is—

1. The process of separating precious metals from matte containing them, which consists in causing an intimate mixture of the 30 matte with metallic iron and subjecting the mixture to a bath of molten metallic lead, substantially as described.

2. The process of separating precious metals from matte containing them, which consists in dissolving metallic iron in molten matte, and then subjecting the mixture to a bath of molten lead, substantially as described.

In testimony whereof I have hereunto subscribed my name.

FRANKLIN R. CARPENTER.

Witnesses:

FRED SMITH,  
GEORGE VICKERS.